

## UNITED STATES PATENT OFFICE

2,300,445

## MORDANTING AGENT

Samuel M. Weisberg, Baltimore, Md., and William E. Stringer, Bronx, N. Y., assignors to Seal-test, Inc., Baltimore, Md., a corporation of Maryland

No Drawing. Application December 4, 1939,  
Serial No. 307,450

8 Claims. (Cl. 8—99)

This invention relates to dyes and relates more particularly to mordants and decomposition or deposition retarding agents for mordants.

Many different types of chemical agents such as, for example, cream of tartar and lactic acid, are used to retard the decomposition and control the rate of deposition of metallic salt mordants in the dyeing of yarn and textiles. Cream of tartar ( $\text{KHC}_4\text{H}_4\text{O}_6$ ) is perhaps the most commonly used of these retarding agents. However, this composition has the serious disadvantage of being expensive and not readily available at all times, inasmuch as it is an imported product.

Lactic acid has not been entirely satisfactory as a decomposition or deposition retarding agent inasmuch as it does not sufficiently retard or slow down the reduction of such mordants as potassium and sodium bichromates.

Attempts have also been made to use salts of lactic acid in conjunction with metallic salt mordants but such attempts consistently have been failures, apparently for the reason that the use of these salts was based on erroneous conceptions of their composition. However, it would be highly desirable to use salts of lactic acid as decomposition or deposition retarders for metallic salt mordants inasmuch as the salts of lactic acid are quite inexpensive as compared with cream of tartar, and at the same time are readily available as a domestic product.

An object of the present invention, accordingly, is to provide metallic mordants containing salts of lactic acid which have a slow and well controlled rate of decomposition or deposition.

Another object of the invention is to provide solutions of salts of lactic acid which act as buffering agents and decomposition or deposition retarders for metallic salt mordants.

Other objects of the invention will become apparent from the description of typical forms of the invention hereinafter.

It has been discovered that the pH value of solutions of salts of lactic acid bear a direct relationship to their ability to act as retarders in the deposition or decomposition of metallic salt mordants, such as, for example, chromium salts, aluminum salts and tin salts, which are well known and commonly used in the art. From a series of tests it has been determined that solutions of lactate salts should be adjusted to a pH value not less than 4.0 in order to obtain the optimum results. Such lactate salt solutions may be used with those mordants with which cream of tartar has previously been used, for example, sodium or potassium bichromate, chrome alum, stannous

chloride, alum and neutral aluminum sulphates. The alkali metal, alkaline earth metal and ammonium salts of lactic acid such as sodium, potassium, calcium, magnesium and ammonium lactates are entirely satisfactory. The retarding effects of these salts will vary somewhat with the type of metallic ion with which the lactate ion is associated. That is, for example, sodium lactate is a more rapid reductant than ammonium lactate, and, accordingly, advantage can be taken of these varying characteristics in controlling the rate of deposition of the metallic mordants.

By way of specific example of the effect of varying the pH value of salts of lactic acid on their properties as buffering and decomposition retarding agents, reference may be had to the following table which discloses a series of tests made with lactic acid, sodium lactate adjusted with lactic acid or sodium hydroxide to different pH values and used in conjunction with a sodium bichromate as a mordant.

## Lactate—Bichromate pH relations

|    | Example                                                                                                             | Initial pH after adding water | pH After addition of chromate | pH After 15 min. boiling | Remarks                                                                                                    |
|----|---------------------------------------------------------------------------------------------------------------------|-------------------------------|-------------------------------|--------------------------|------------------------------------------------------------------------------------------------------------|
| 30 | #1                                                                                                                  |                               |                               |                          |                                                                                                            |
|    | Water 100 cc.—<br>Lactic acid (50%) 2.5 gms.—<br>Sodium dichromate 2.5 gms.—                                        | 2.1                           | 2.2                           | 6.3                      | Reduction very rapid; brown gelatinous precipitate formed.                                                 |
| 35 | #2                                                                                                                  |                               |                               |                          |                                                                                                            |
|    | Water 100 cc.—<br>Sodium lactate (50%) adjusted to pH 4.0 with lactic acid 2.5 gms.—<br>Sodium dichromate 2.5 gms.— | 3.5                           | 3.5                           | 6.3                      | Reduction rapid but not as rapid as for (1). Some brown gelatinous precipitate but not as much as for (1). |
| 40 | #3                                                                                                                  |                               |                               |                          |                                                                                                            |
|    | Like #2 but sodium lactate adjusted with lactic acid to pH 5.5.                                                     | 5.0                           | 4.8                           | 6.3                      | Reduction rate moderate. No precipitate.                                                                   |
| 45 | #4                                                                                                                  |                               |                               |                          |                                                                                                            |
|    | Like #2 but sodium lactate adjusted to pH 7.0 with lactic acid.                                                     | 7.0                           | 5.1                           | 6.3                      | Do.                                                                                                        |
| 50 | #5                                                                                                                  |                               |                               |                          |                                                                                                            |
|    | Like #2 but sodium lactate adjusted to pH 10.0 with sodium hydroxide.                                               | 8.7                           | 5.0                           | 6.3                      | Do.                                                                                                        |

It will be seen from the above table that lactic

acid or sodium lactate and sodium bichromate solutions having a pH value of lower than 4.0 are entirely unsatisfactory because of excessively rapid rate of reduction of such mordants and the formation of precipitates.

On the other hand, Examples 3 to 5, inclusive, show that so long as the initial pH value of the sodium lactate solution is above 4.0 the reduction rate will be moderate, no precipitate will be formed, and these compositions will result in satisfactory dyeing operations.

It will be apparent also from the above table that sodium lactate has an extremely high buffering action inasmuch as in Example #5, the sodium lactate solution which was initially adjusted to pH 10.0, upon mixture with sodium bichromate resulted in a solution having a pH value of 5.0, which is very close to the pH value of the solutions disclosed in Examples 3 and 4. It should be understood, of course, that the pH values indicated in column 3 of the above table (pH value after addition of chromates) are the pH values of the mordant alone and not the pH values of the mordant in the presence of a fabric or other material being dyed. Because of this high buffering action of sodium lactate, excessive amounts of alkali are required to produce solutions having pH values exceeding 10.0 and it is not practical to operate above this pH value because of the expense involved. Therefore, for practical purposes, lactate solutions having a pH value between 4 and 10 are entirely satisfactory.

The value of lactate solutions has been established by conducting dyeing tests upon wool. In every instance excellent dyeing results were obtained, using mixtures of sodium lactate adjusted to a pH value exceeding 4.0 and sodium bichromate.

It will be apparent that solutions of salts of lactic acid are highly effective buffering agents and decomposition retarders and have a wide field of use in the dyeing industry. It will be understood, moreover, that excellent control over the

action of mordants is obtained by the use of such salts, not only by varying their concentration but by utilizing salts of lactic acid which have different metallic ions. Accordingly, it will be understood that there may be variations in the proportions of such salts and they may be used in different combinations with various metallic mordants without departing from the invention. The specific examples given above, therefore, should be considered as illustrative only and not as limiting the scope of the following claims.

We claim:

1. A mordant comprising a solution having a pH value between about 4.8 and 5.1 containing a chromium salt and a salt of lactic acid.
2. A mordant comprising a solution having a pH value between about 4.8 and 5.1 containing sodium bichromate and a salt of lactic acid.
3. A mordant comprising an aqueous solution of a chromate and a salt of lactic acid in about equal proportions, said solution having a pH value between about 4.8 and 5.1.
4. A mordant comprising an aqueous solution of a metallic salt mordant and a salt of lactic acid, said solution having a pH value between about 4.8 and 5.1.
5. A mordant comprising a solution having a pH value between about 4.8 and 5.1 containing a chromium salt and sodium lactate.
6. A mordant comprising a solution having a pH value between about 4.8 and 5.1 containing sodium bichromate and sodium lactate.
7. A mordant comprising an aqueous solution of a chromate and sodium lactate in about equal proportions, said solution having a pH value between about 4.8 and 5.1.
8. A mordant comprising an aqueous solution of a metallic salt mordant and sodium lactate, said solution having a pH value between about 4.8 and 5.1.

SAMUEL M. WEISBERG.  
WILLIAM E. STRINGER.